

May 2, 1933.

Y. UEKI

1,907,224

APPARATUS FOR ELECTRICALLY COATING THE BORE OF CARBON  
BRUSHES FOR ATTACHING THE LEAD WIRE WITH METAL  
Filed April 25, 1931

Fig. 1.



Fig. 2.



Fig. 3.  
b  
a



Fig. 4.  
b  
a



Fig. 5.  
b  
a



Inventor  
Yoshigoro Ueki  
By Raymond O. Herlihy  
Attorney

## UNITED STATES PATENT OFFICE

YOSHIGORO UEKI, OF EBARA GUN, TOKYO, JAPAN

APPARATUS FOR ELECTRICALLY COATING THE BORE OF CARBON BRUSHES FOR  
ATTACHING THE LEAD WIRE WITH METAL

Application filed April 25, 1931, Serial No. 532,882, and in Japan May 8, 1930.

The present invention relates to improvements in a method and apparatus for electrically coating with metal the bore into which a lead wire is to be secured in carbon brushes and the like. In copper coating the bore, electrically, according to the present invention, thin rubber or like plates of height and width equal to the carbon brushes, and provided with electrodes at the portions corresponding to the bore of brushes, are alternately piled in series with the carbon brushes and tightly clamped together. This forms baths at the bore of the carbon brushes, in which bores an electrical coating is desired.

15 The object of the invention is to electrically coat the bore of carbon brushes, without dipping the same in an electric plating bath. Another object of the invention is to avoid the change of brush size, when metal plated 20 at unuseful portions. A further object of the invention is to perfectly coat the bore with copper, without affecting the quality of the brush, and to reduce electric resistance at the portion where the lead wire is to be 25 fitted.

Hitherto, it has been common to copperplate the bore of carbon brushes to reduce electric resistance at the contact part of the lead wire; the upper part of the carbon brush being 30 dipped into an electrolytic bath for electrically coating the inner surface of the lead wire receiving bore. According to said process, the brush is inevitably coated also on parts other than the bore, the size of the brush being 35 thereby changed, so that this process is inapplicable in cases where the allowable difference in the size of brushes is restricted, for instance, within five thousandths of an inch. It has also been proposed to coat brushes 40 with paraffin or the like, on parts other than the bore, to prevent metal from being coated thereon. However, the nature of the brush is considerably affected by said paraffin coating and a rather harmful effect is induced 45 thereby.

According to the present invention, the bore of carbon brushes can be perfectly coated with metal without changing the size or affecting the nature of the brush. The invention is characterized in that the bore itself

constitutes the electric bath, and only the lead wire receiving bore may be perfectly coated with metal easily and rapidly.

The invention is fully described with reference to the accompanying drawing in which:

55 Figure 1 is a vertical sectional view of the improved apparatus showing the bores filled with solution, for carrying out the process,

Figure 2 is an elevation showing a rubber plate provided with an electrode at its top, and adapted to be alternately piled in a series with the brushes, and

60 Figures 3, 4 and 5 show, in bracketed arrangement, elevations and side views, respectively, of various forms of bores formed in 65 brushes.

The same reference characters designate corresponding parts throughout the drawing.

Referring now to the apparatus of Figure 1, wherein several brushes are shown having 70 their bores filled with coating solution, C designates the carbon brushes to be treated, 1 and 2 designates feed wires connected to a generator, or other source of electricity. 3 designates copper electrodes connected to the 75 positive terminal of the generator. 5 designates rubber, cork or similar plates provided with copper electrodes 3 and copper washers 80 9. 6 designates a screw bolt for tightening the runner plates closely to the brushes C 80 alternately piled in a series with the plates 5. 8 designates the bores formed at the upper 85 part of the brushes C, for attaching the lead wire therein, and filled with coating solution Q for carrying out the process.

Fig. 2 shows in elevation a rubber plate 5. At the upper edge of said rubber plates a copper electrode 3 is inserted and copper washers are attached at both sides, through 90 the centre of which apertures 4 are formed for passage of the coating solution.

Figs. 3, 4 and 5 show various forms of bores for attaching lead wires, a as front elevations and b as side elevations. 8 designates the bores for fitting the lead wire there- 95 in and 11 the recesses for receiving the washers. Said bores and recesses are filled with coating solution.

In carrying out the invention carbon brushes finished to a desired size are alter- 100

nately piled in series with rubber plates 5, keeping the bores in line, and the screw bolt 6 rotated to tightly compress the whole together. In the recesses formed by the bores 5 of the brushes, forming plating baths, is poured a solution containing pure copper sulphate 453 grms., sulphuric acid 23 grms., zinc acetate 23 grms. and pure water 9 litres. Keeping the temperature of the solution at 10 20° to 40° C. an electric current of 1 to 3.2 volts is passed at the rate of 0.8 to 2.4 amperes per square millimetre of the coating surface. The current is held for about 10 minutes, whereby a copper coating of two thousandths 15 to three thousandths of an inch thick is obtained inside the bore.

When the lead wire is fitted in the bore of the brush, as treated above, it is kept in close contact therein and electric resistance at said 20 contact part is reduced from one half to one third, as compared with those not coated with metal in the bore. The treatment may be easily and rapidly performed without affecting the size and quality of the carbon brush.

25 I declare that what I claim is:—

An apparatus for electroplating carbon articles, comprising means to press together a number of stacked carbon articles, insulating members disposed between each carbon 30 article of the pressed stack, a connector associated with each insulating member and extending on a portion of two sides of this member flush with the surface thereof, and an electric current source suitably connected to 35 the carbon pack and the connectors, whereby an electrolytic liquid introduced in cavities of the carbon articles and in contact with the extending portions of the connectors is decomposed and caused to deposit a layer of 40 metal inside the said cavities of the carbon articles.

In testimony wherefor I have affixed signature.

YOSHIGORO UEKI.

45

50

55

60

65